

Oct. 17, 1939.

M. J. UDY

2,176,687

CHROME ALLOY MAKING

Filed Jan. 22, 1938

2 Sheets-Sheet 1

Fig. 1,



INVENTOR  
MARVIN J. UDY

BY

Pennie, Davis, Marvin & Edmonds  
ATTORNEYS

Oct. 17, 1939.

M. J. UDY

2,176,687

CHROME ALLOY MAKING

Filed Jan. 22, 1938

2 Sheets-Sheet 2

Fig. 2.



INVENTOR

MARVIN J. UDY

BY

Pennie, Davis, Marvin and Edmonds  
ATTORNEYS

## UNITED STATES PATENT OFFICE

2,176,687

## CHROME ALLOY MAKING

Marvin J. Udy, Niagara Falls, N. Y.

Application January 22, 1938, Serial No. 186,466

31 Claims. (Cl. 75—27)

This invention or discovery relates to chrome alloy making; and it comprises manufacture of a composition for use in making chrome iron alloys, said composition being a mixture of pulverulent substantially carbon-free and completely oxidized ferrochromium with pulverulent ferrochrome metal low in carbon and high in silicon, in proportions enabling the composition to undergo internal exothermic reactions forming low carbon ferrochromium metal to be supplied to a steel or iron bath in any ratio; and it further comprises a method of utilizing chromite ores of any grade in making alloy steels wherein ferrochromium metal made from chromite by total reduction with carbon and rich in carbon is subjected to an oxidizing roast in the presence of lime thereby eliminating carbon, the oxidized product in pulverulent form is admixed with a pulverulent metal containing chromium, iron and silicon in high proportion, said metal being formed by remelting ferrochromium with silica and carbon and the admixture is added to molten iron or steel to form the desired alloy; all as more fully hereinafter set forth and as claimed.

Chromium alloys of iron and steel have reached great commercial importance for various purposes, particularly as corrosion-resistant or rustless iron or stainless steel and as oxidation-resistant and high strength ferrous metals generally. For the most part the chromium in these alloys is supplied by ferrochromium made from chromite ores and diluted, so to speak, with iron; other alloying metals, nickel, vanadium, molybdenum, tungsten, etc., being often added in small quantities. The chromium content may range from a fraction of a per cent to above 30 per cent; iron being the major component of the alloy. Processes have been proposed for making chrome steel direct from chromite ores. For various reasons such "direct" processes have not proved successful. In practice, for the most part, the ore is first reduced to ferrochromium as an intermediate alloy supplying chromium for the finished steel or iron alloy.

In utilizing ferrochromium as source of chromium for these alloys, a large problem in the industry arises from a requirement that the alloy shall be extremely low in carbon content; a usual maximum of tolerance being 0.2 per cent. Carbon lower than 0.05 per cent of the alloy is often desirable. Generally speaking, for most technical uses, the lower the carbon content, the better is the quality of the alloy. Ferrochromium always carries carbon. To meet the low carbon requirement in the finished alloy, not only must

the steel or iron forming the major part of the alloy be carefully refined but means must be found to avoid carbon being carried into the steel by the ferrochromium serving as source of chromium for the alloy.

Carbon elimination in chromium metallurgy entails great expense. The industry is forced in great measure to use a special low carbon ferrochromium made by reducing chromite ores with non-carbonaceous reducing agents; in which the cost per unit of chromium is double that for chromium in the high carbon grades of ferrochromium produced by the usual electric smelting of chromite ores with carbon (coke) as a reducing agent. It has also been considered necessary to use ferrochromium of the highest possible chromium content as well as low in carbon; the present standard being 70 per cent chromium or a ratio of chromium to iron of 2.33:1. For this it has been necessary to comb the globe for high grade or low iron chromites, leaving unutilized plentiful supplies, both domestic and foreign, of good ores too high in iron to yield standard marketable ferrochromium; metal with the high chromium content considered necessary in ferrochromium used to supply chromium for the alloy steel and iron. The industry, to avoid carbon in the final alloy, has to use a low carbon high grade ferrochromium made from the rare high grade ores and then to dilute this metal with iron in making commercial alloys carrying minor percentages of chromium. So the industry labors under the fundamental economic disadvantage of standing the cost of a 70 per cent chromium low carbon metal which is diluted with iron to an alloy containing usually less than 30 per cent chromium.

In my Patent 2,098,176, November 2, 1937, I have described and claimed manufacture of a synthetic chromite ore containing calcium chromite replacing ferrous chromite of the natural ore, by selective reduction of iron from ferrous chromite ore in the presence of lime. By the invention of said patent substantially complete control is afforded of the chromium-iron ratio in chromite ores and thus in the ferrochromium subsequently produced. This permits utilizing in chromium metallurgy for making marketable high grade ferrochromium, the low grade (high iron) chromite ores hitherto unavailable for such use.

In the present invention I depart from the practice of making commercial chrome steels by directly adding commercial ferrochromium of the highest possible grade to molten iron or steel.

Instead, I add to the molten bath a particular two-component mixture of oxides with metal containing silicon in proportion sufficient to reduce the oxides by exothermic action, giving a substantially carbon-free metal containing chromium and iron. The oxidized component of the mixture is made by roasting metal produced by total reduction of a chromite ore with carbon. In roasting the carbon disappears and oxides of chromium and iron are reproduced. This roasted material is one component of my mixture. The other component is a metal rich in silicon and low in carbon produced by remelting a similar total-reduction metal, remelting being with silica and carbon. The two components are mixed in such proportions that the silicon in one component reduces the oxides of iron and chromium in the other with evolution of heat. Such a composition on mixture with molten iron undergoes reaction with the production of a chromium iron alloy of any ratio of chromium to iron desired in commercial alloys. In the chromite ore used in producing the two components, the ratio of chromium to iron is, within limits, immaterial.

Other things being equal, the heat evolution in the two component mixture increases with an increase in the proportion of iron in the oxide component and vice versa. Therefore low grade ores with a high ratio of iron to chromium are desirable in making the oxide component.

In practice the exothermic mixture contains as a third component enough lime to form a basic silicate slag with the silica formed from the silicon in the reaction. The lime containing composition when added to a molten steel bath supplies chromium in any desired ratio and at the same time contributes heat to the bath. The silica formed in the action combines with the lime to form a low melting basic slag which can be of relatively low volume in relation to the iron-chromium metal formed in the action. The lime combining with silica adds somewhat to the heat of evolution. By proper proportioning of the mixture components, the heat of the exothermic reaction may contribute a great part or all of the heat required to bring to fusion both the lime silicate slag and the metal which are products of the reaction. The conversion of silicon to silica may be complete, with sufficient lime in admixture to form a silicate containing lime in excess of an equimolecular ratio to the silica. A ratio of 1.5:1 for example, effects completion of the exothermic reaction. With  $\text{CaO}/\text{SiO}_2$  ratios between 1 and 2 the Si content of the metal product is under substantially complete control.

In utilizing the exothermic mixture for making alloy steel, it is possible to ignite the mixture in a hot furnace and to add the hot products of the silico-thermic reaction to a bath of refined molten steel in an open hearth furnace.

According to the invention there is provided from low grade chromite ores a composition useful as an intermediate material for making chromium alloy steels in the open hearth furnace. The intermediate may carry into the steel from 90 to 95 per cent of the total chromium of the ores used; the silicon in the exothermic mixture being in proportion to reduce both the chromium and the iron of the oxidized component; the proportion of lime in the mixture sufficient to form a basic silicate slag contributing as I have found, to substantially complete reduction of the oxides without more than a slight excess of silicon going into the finished alloy steel. In a short period of time the basic slag refines silicon out of the metal.

Commercial alloyed steel (iron) is made by diluting with molten iron the metal product of the internal exothermic reaction; the added iron being sufficient to establish the desired chromium ratio in the finished alloy.

In a copending application Serial No. 185,417, filed September 23, 1937, I describe methods of oxidizing ferrochromium to calcium iron chromite. This oxidation of the metal results in substantially complete elimination of the carbon contained therein and is advantageously carried on in the presence of a relatively large quantity of lime. The oxidation product composed of lime, ferric oxide and chromic oxide which is conveniently termed calcium ferrichromite, may be used to great advantage as the oxidized component of the stated composition. It is advantageous if it contains the amount of lime required to form a basic silicate, as described, with the silica produced from the second component. Basicity aids the oxidation of Si to  $\text{SiO}_2$ .

In roasting ferrochromium with lime and a little soda ash to total oxidation of the metals and elimination of carbon, as described in my acknowledged prior application, I have found it advantageous to oxidize a substantial proportion of the chromium to  $\text{CrO}_3$  and to leave in the oxidized material a substantial content of chromate. So doing, a mixture of the chromate-containing calcium ferrichromite with siliconized ferrochromium may be made to convert itself into molten ferrochrome metal and molten basic silicate slag.

It is possible to fully roast ferrochromium in the presence of a base to ferric oxide and chromate of the base. This is described in my copending application Serial No. 177,365, filed November 30, 1937. With lime alone serving as the base the oxidation of chromium to chromate requires several hours of roasting, but with soda present in adequate amount the conversion to chromate may be complete in half an hour at or somewhat below 1000° C. It is possible to control the rate and degree of conversion to chromate in roasting chromium and lime by the quantity of soda present and by regulation of the temperature.

Roasting at temperatures well under 1000° C. with no soda ash or less than one per cent of soda in the roasting charge converts the chromium mostly to calcium chromate without complete oxidation and elimination of carbon from the ferrochrome metal in a reasonable length of time. Above 1000° the carbon is eliminated but the chromate breaks down to chromite. As the soda is increased the temperature can be raised without breaking down the chromate and the carbon can be completely eliminated without raising the temperature. Additions of soda in amounts above one per cent of the charge or two per cent of the metal permits regulation of the temperature to control the ratio of chromate to chromite ( $\text{CrO}_3$  to  $\text{Cr}_2\text{O}_3$ ) in the oxidized product. I have found for example that addition to a roasting mix of ferrochromium and lime of soda ash ( $\text{Na}_2\text{CO}_3$ ) in the amount of 5 to 10 per cent by weight of the ferrochromium metal results in 50 per cent conversion to chromate in a short time with total elimination of carbon and oxidation of all the metal when the temperature of roasting is held at 1000° C.; the remaining chromium being oxidized to  $\text{Cr}_2\text{O}_3$  appearing as calcium chromite. This 50-50 oxidation of chromium to chromite and chromate gives an oxidized material capable of a highly exothermic reaction with siliconized ferrochromium. Such a compound of  $\text{CaO}$ ,  $\text{Fe}_2\text{O}_3$ ,  $\text{Cr}_2\text{O}_3$  and  $\text{CrO}_3$  containing a small amount of

Na<sub>2</sub>O from the soda ash and made from ferro-chromium by roasting in air, is a highly advantageous material to be admixed with ferrosilicon or ferrochrome silicon to form the exothermic or silico-thermic material of the present invention.

The roasting operation can be carried on in an open hearth or reverberatory furnace with mechanical rabbling or in a rotary kiln. Limestone may be used in the roasting mix to supply lime. A little soda, in the order of 2 to 10 per cent of the metal, besides controlling the conversion to chromate greatly promotes the oxidation of the chromium to chromite. The soda may be added to the roasting mix in the form of sodium chromate. The roasting may be made to yield any desired ratio of CrO<sub>3</sub> to Cr<sub>2</sub>O<sub>3</sub> in the oxidized product.

For siliconizing high carbon ferrochromium, a mixture of crushed or granular metal with 20 silica rock (quartzite) and coke may be charged continuously into a submerged arc electric furnace and a metal siliconized to a low carbon content is tapped from the furnace; high silicon content in the tapped metal replacing the carbon content of the charged ferrochromium. The silicon content may be as high as desired, up to 25 per cent, for example. This operation is similar to that of making ferrosilicon; the high carbon ferrochrome taking the place of scrap iron.

An exothermic mixture of calcium ferrichromite containing chromate with ferrochrome-silicon containing a slight excess of silicon over the quantity required to reduce the iron and chromium oxides is a highly advantageous material for supplying to molten refined steel the chromium required for a finished alloy. A calcium ferrichromite made by total oxidation of high carbon ferrochromium in the presence of much lime and some soda, the latter serving as a wetting agent for the ferrochromium undergoing oxidation, as described in the companion application, is substantially free of carbon. And a ferrochrome-silicon made by smelting high carbon ferrochromium with silica and carbon to a high silicon content may also be substantially free of carbon. A mixture of the two within the purview of the present invention, added to a steel bath, supplies substantially carbon-free iron-chromium metal together with heat to be used for melting the lime silicate slag and metal formed in reduction by silicon. Thus chromium is supplied to the steel with substantially complete elimination of the carbon of ferrochromium.

In adding a two-component mixture of oxidized and siliconized ferrochromium to the steel bath, as described, it is possible to so proportion the two reagents as to minimize the accompanying slag production. The amount of slag relative to the metal chromium is dependent upon the proportion of iron oxide introduced with the chromium oxides in the oxide component and reduced by the silicon of the other component. This in turn depends upon the chromium-iron ratio in the oxidized ferrochromium and in the chromite ores from which it is made by total reduction. While the higher grade materials (of lower iron ratios) give oxidized and siliconized products involving smaller slag additions to the steel furnace, it has been found that the larger slag additions per unit of chromium associated with the use of low grade chromites and ferrochromiums of high iron ratios are by no means prohibitive. In fact, it is possible to use the lowest grade ores as source of the ferrochromium,

both that which is oxidized and that which is siliconized. I have even used, for example, chromiferous iron ores with 2 to 3 per cent chromium content; with a ratio to the iron content of 1:20. This is described in an accompanying application.

Using chromite ores of sub-standard grade with total reduction to high carbon ferrochromium followed by portional oxidation and siliconizing of the ferrochromium, the proportions of oxidized and siliconized product finely divided and admixed for introduction into the steel furnace determine the ratio of slag added with the iron-chromium metal. A major proportion of the oxidized product admixed with a minor proportion of the siliconized product gives excellent results. This proportioning permits addition of silicon to ferrochromium in a ratio sufficient for nearly complete absence of carbon from the ferrochrome silicon. The lower the proportion in the siliconized product of the total iron and chromium in the mixture, the higher is the percentage of silicon in this product required to reduce the iron and chromium of the oxidized product. However, it has been found in utilizing low grade ores that the lower chromium content of the high carbon ferrochromium permits complete carbon removal with addition of a smaller percentage of silicon to the metal than is required for higher grade ferrochromium. For example, a ferrochromium of a Cr-Fe ratio less than 1:1, as I have found, has the carbon content lowered to less than 0.10 per cent by smelting with silica and carbon to a silicon content of 40 per cent in the ferrochrome silicon product. This compares with considerably higher percentages of silicon required to lower the carbon content below 0.10 per cent in ferrochrome alloys having standard Cr-Fe ratios above 2:1. There is thus an incidental advantage in using sub-standard ferrochromium made from low grade chromites.

In utilizing mixtures of oxidized and siliconized ferrochromium made from low grade ores of chromium-iron ratios between 1 and 2 to 1, exothermic actions in the mixture may be exemplified in chemical equations:



Equation 1 represents action in a mixture of oxidized and siliconized ferrochromium both having a Cr-Fe ratio less than 1:1; the proportions of oxidized and siliconized ferrochromium taking part in the reaction being 1:1.5 or 40:60 per cent of the original 1:1 ferrochromium, 40 per cent being oxidized and combined with lime as calcium ferrichromite and 60 per cent being siliconized to a 20 per cent silicon content; the products being low carbon ferrochromium and a calcium silicate slag containing 4CaO to 3SiO<sub>2</sub> and in a weight ratio of 75 per cent of the ferrochromium; the heat developed in the reaction being estimated from available data as 109,000 calories or 2590 centigrade units per pound silicon oxidized. There is an ample margin of heat over that required to melt the slag; (something under 5 pounds slag per pound silicon). The production of metal in the reaction is over 75 pounds per pound silicon oxidized.

In Equation 2 the chromium-iron ratio of the oxidized and siliconized ferrochromium is 1.85, the proportion of oxidized and siliconized ferrochromium is 73:27 and the silicon content of the ferrochrome silicon in the mixture is 51 per cent. The slag to metal ratio is 1.37. The heat set free in the reaction may be estimated at 144,700 calories, or 2300 centigrade units per pound of silicon oxidized; an amount of heat ample for raising 5 pounds slag per pound of silicon to the temperature of a steel furnace. The production of metal is nearly 3.5 pounds per pound Si.

Equation 3 illustrates silico-thermic reduction of calcium chromate by ferrochrome silicon (50 per cent Si) with production of 2.20 pounds metal and 4 pounds slag per pound silicon with an estimated heat evolution of 4000 centigrade units; which appears in excess by some 60 per cent over the heat used in melting the metal and slag products of the reaction. The equation illustrates the quantitative effect of chromate contained in the oxidized component in supplying heat for making the reacting admixture with the siliconized component fully exothermic when ignited in a hot furnace or when added to a bath of molten steel as in an open hearth steel furnace.

If in roasting ferrochromium to make the oxidized or oxygenated component of the silico-thermic mixture, all or the greater part of the chromium is converted to chromate the heat of the reaction is greatly increased and the silicon content of the siliconized component may be lessened. However, the excess heat may be utilized in adding to the heat of the steel bath.

While a lower silicon content in the siliconized low carbon ferrochromium permits a higher proportion of this product in admixture with oxidized ferrochromium, it is sometimes advantageous to lower the proportion of ferrochrome-silicon in the mixture and to increase the silicon percentage, thus supplying additional silicon for reduction of the higher proportion of oxides in the mixture. This effects additional heat development when the mixture is fed to the steel furnace, the additional heat being accompanied by an increased slag ratio. There is a net gain of heat delivered to the furnace by the internal exothermic reaction of which the mixture is capable, the delivery of heat per unit weight of the material being in direct proportion to the percentage content of reducible oxides and the equivalent silicon for reduction.

An important advantage of the invention as described is that it results in being able to prepare in the open hearth steel furnace alloy steels of greater chromium content than has heretofore been practicable. These alloys carrying from 12 to 18 per cent chromium and above can now be made in the open hearth, utilizing the present invention. For making such relatively high chromium alloys the electric furnace is no longer necessary. But it may be used, when desired.

The exothermic mixture may be ignited in a separate furnace and molten metal and slag run into the open hearth. The effect is that of adding molten low carbon ferrochromium.

Another advantage of the method is that alloying metals, other than chromium, may be added as oxides to the exothermic mixture or in metallic form to the ferrochrome silicon component. As an example of the latter modification, nickel silicate ore may be utilized as source of silica for

siliconizing high carbon ferrochromium, this incorporating nickel in the metal in addition to iron and chromium as nickel-ferrochrome silicon. Oxides of nickel, vanadium, molybdenum, etc., may be made part of the oxidized component of the mixture fed to the steel bath, and thus be reduced by silicon to metal which is thus added to the steel with the chromium supplied by the mixture.

In practice of the invention, a number of modifications are possible. The exothermic mixture of oxidized and siliconized ferrochromium may be so compounded as to form the equivalent of ferrochromium having any desired carbon content within the usual commercial ranges. The mixture of oxidized and siliconized ferrochromium can be so made as to yield a substantially carbon-free metal. By adding into the mixture a proportion of finely ground high carbon ferrochromium the metal product can be made to contain a corresponding percentage of carbon. As I have found, it is desirable to have in the mixture silicon equivalent to the chromium and iron oxides therein. Then addition to the mixture of high carbon ferrochromium puts carbon into the metal. With sufficient lime present to convert the silica formed in the reduction into calcium silicates, little or no silica is reduced by carbon. This affords complete control of the carbon content of the metal product. In a chromate mixture with silicon insufficient for the reduction, residual carbon in the siliconized metal is oxidized and removed by reduction of the oxide component; heat absorbed in this reduction being supplied by the silicon reaction.

In siliconizing high carbon ferrochromium at 1500 to 1600° C. in a submerged arc electric furnace, a comparatively small amount of carbon in the metal is replaced by adding a much larger amount of silicon. In this operation, as above noted, it is advantageous to have a relatively low chromium-iron ratio in the metal. A high carbon ferrochromium made from low grade ores requires a relatively small addition of silicon to eliminate carbon. In utilizing low grade ores it is possible to control the carbon content of the finished steel by varying the silicon percentage added to the ferrochromium so as to leave more or less carbon in the metal component of the silico-thermic mixture added to the steel.

In another modification of the silico-thermic mixture the silicon content is sufficient to reduce the chromium of the oxidized ferrochromium component and iron oxide in this component is reduced by carbon either in high carbon ferrochromium added to the mixture or present as residual carbon in the siliconized component.

If desired, an oxidizer such as sodium chlorate or nitrate may be incorporated in the mixture with excess silicon to be oxidized for additional thermicity.

As a general rule it is advantageous, as stated, to utilize the lower grade chromite ores for making both the oxidized and the siliconized ferrochromium in the silico-thermic mixture. However, any desired grade of ore may be used for making either component. It may be desirable for example, to siliconize a low grade ferrochromium and to oxidize a high chromium metal to chromate and  $Fe_2O_3$ , in making the silico-thermic mixture.

In siliconizing ferrochromium, and particularly the lower grade materials to relatively low

silicon percentages, it is possible to carry on the operation in a blast furnace such as used commonly for making pig iron.

In a specific embodiment of my invention I have made a mixture of oxidized with siliconized ferrochromium in a ratio of 61:39 from a ferrochromium containing 66.4 per cent chromium, 4.66 per cent carbon, 2 per cent silicon and 27 per cent iron.

- 10 In oxidizing this metal 100 parts were intimately mixed and finely ground in a ball mill with 115 parts lime, CaO, and 6 parts soda ash, Na<sub>2</sub>CO<sub>3</sub> and this finely ground mixture was roasted in a gas fired rotary furnace at temperatures from 700 to 1100° C. The roasted product was a chromated calcium ferrichromite analyzing as follows:

Per cent

|                                |      |
|--------------------------------|------|
| Cr <sub>2</sub> O <sub>3</sub> | 14.8 |
| CrO <sub>3</sub>               | 22.9 |
| Fe <sub>2</sub> O <sub>3</sub> | 13.4 |
| SiO <sub>2</sub>               | 8.4  |
| CaO                            | 38.2 |
| Na <sub>2</sub> O              | 2.0  |

- 25 The proportion of chromium as chromate is 54 per cent.

The above high carbon ferrochrome metal was siliconized by smelting in a submerged arc furnace with quartzite and coke to a silicon content of 50 per cent with 35 per cent Cr and 15 Fe. 117 parts of this ferrochrome silicon (equivalent to 63 parts of the original metal) were pulverized and intimately admixed with the 271 parts of ferrichromate produced by oxidation as above described of 100 parts of high carbon metal and with 72 parts of lime in a ball mill.

40 This mixture was quickly fed to a red hot steel furnace and thereby ignited. The mixture reacted exothermically and converted itself to 146 parts of low carbon ferrochromium molten metal analzing 70 per cent chromium, 0.05 per cent carbon and silicon under 1 per cent with approximately 312 parts molten calcium silicate slag containing lime and silica in a ratio of 1.5 to 1 and 1.6 per cent chromium. The recovery of chromium from the original high carbon metal was 95 per cent.

45 Molten iron can be added to this low carbon metal in any ratio to make a finished alloy of desired chromium content.

In a specific example of my invention utilizing a low grade ore analzing as follows

Per cent

|                                |       |
|--------------------------------|-------|
| Cr <sub>2</sub> O <sub>3</sub> | 13.75 |
| Iron oxides as FeO             | 12.00 |
| MgO                            | 21.18 |
| Al <sub>2</sub> O <sub>3</sub> | 2.02  |
| SiO <sub>2</sub>               | 35.70 |
| CO <sub>2</sub>                | 14.30 |

50 I smelt this ore in a submerged arc furnace in continuous operation by the process described in my copending application Serial No. 165,954, and produce a metal of the following composition:

Per cent

|    |    |
|----|----|
| Cr | 42 |
| Fe | 48 |
| C  | 7  |
| Si | 3  |

55 I roast in air 100 parts of this metal with 100 parts of lime. The roasting is at a temperature somewhat under 1000° C. for a time and then at 700° to 1100° C. From this

roast, 236.4 parts of calcium ferrichromite are obtained analyzing as follows

|                                | Per cent |
|--------------------------------|----------|
| Cr <sub>2</sub> O <sub>3</sub> | 25.9     |
| Fe <sub>2</sub> O <sub>3</sub> | 29.0     |
| SiO <sub>2</sub>               | 2.7      |
| CaO                            | 42.2     |
| C                              | .02      |

10 I smelt 36 parts of the above metal with silica and coke in a submerged arc furnace and produce 72 parts ferrochrome silicon containing 50 per cent Si, 23.4 per cent Cr, 26.6 per cent Fe with 0.04 per cent carbon.

15 For making low carbon metal I mix or briquette for reaction on a steel bath, or for separate reaction to produce low carbon ferrochrome, the 236.4 parts of calcium ferrichromite and 72 parts of the 50 per cent ferrochrome silicon ground to 100 mesh or finer. In the internal reaction of this 20 mixture there is produced 126 parts of metal analzing 46.5 per cent Cr and 53.4 per cent Fe, with less than 0.10 per cent carbon. With this metal there is produced in the reaction 186 parts of calcium silicate slag containing about 5 per cent Cr<sub>2</sub>O<sub>3</sub>. If made on the steel bath the metal 25 enters the steel to supply chromium in the ratio desired. If reacted to produce ferrochrome, excess silicon may be used in the mixture with sodium nitrate or chloride to produce additional 30 heat. In this example, 92 per cent of the original ferrochromium appears in the metal product of the exothermic reaction.

35 If I wish to produce, for example, the equivalent of 1.5 to 2 per cent carbon grade ferrochrome, I mix and react the 236 pounds of ferrichromite, 72 pounds of ferrochrome silicon and 35 pounds of the original high carbon ferrochromium containing 7 per cent carbon and produced from the ore as described. I thus make 160.9 40 pounds of metal containing 46 per cent chromium and 51 per cent iron with 0.65 per cent Si and 1.52 per cent C.

45 In a third example of the invention, two different ores are used having the following analyses

| Ore No. 1                      |          |          | Ore No. 2 |                                |          |
|--------------------------------|----------|----------|-----------|--------------------------------|----------|
|                                | Per cent | Per cent |           | Per cent                       | Per cent |
| Cr <sub>2</sub> O <sub>3</sub> | 38.40    | Cr       | 22.95     | Cr <sub>2</sub> O <sub>3</sub> | 43.00    |
| FeO                            | 12.61    | Fe       | 9.85      | FeO                            | 25.00    |
| CaO                            | 1.90     |          |           | CaO                            | Trace    |
| MgO                            | 14.31    |          |           | MgO                            | 10.80    |
| Al <sub>2</sub> O <sub>3</sub> | 22.95    |          |           | Al <sub>2</sub> O <sub>3</sub> | 15.60    |
| SiO <sub>2</sub>               | 6.50     |          |           | SiO <sub>2</sub>               | 3.80     |

The Cr/Fe ratio in ore No. 1 is 2.84 and in ore No. 2 is 1.52.

50 I first beneficiate 100 parts of No. 2 ore by replacement of FeO with CaO as described in my Patent No. 2,098,176, and produce 27.7 parts of metal analzing 31.7 per cent Cr, 63.2 per cent Fe and 5 per cent C, together with something less than 100 parts of calcium chromite ore containing 20.7 parts chromium and 1.94 parts iron.

55 I next smelt the altered calcium chromite ore with 100 parts of ore No. 1 in a submerged arc furnace and produce 59 parts of metal analzing 70 per cent Cr, 19.9 per cent, C 7 per cent and Si 3 per cent. The slag goes to waste carrying with it the ore gangue refractories, MgO and Al<sub>2</sub>O<sub>3</sub> out of the system.

60 I roast 59 parts of this metal with 59 parts

of lime to produce 139.6 parts calcium ferrichromite analyzing:

|                                | Per cent |
|--------------------------------|----------|
| Cr <sub>2</sub> O <sub>3</sub> | 43.2     |
| Fe <sub>2</sub> O <sub>3</sub> | 11.9     |
| CaO                            | 45.0     |
| Carbon, less than              | 0.02     |

I smelt 20 parts of the 27 parts of metal obtained in altering No. 2 ore with silica and coke in a submerged arc furnace and produce 38 parts of ferrochrome silicon analyzing 50 per cent Si, 16.7 per cent Cr, 32.2 per cent Fe and 0.04 per cent C. I then mix this ferrochrome silicon with the 139 parts of calcium ferrichromite to produce by exothermic reaction approximately 70 parts of low carbon ferrochromium analyzing 65 per cent Cr and 34.8 per cent Fe. This metal runs about 0.03 per cent in carbon content.

If to the 139 parts of ferrichromite and 38 parts ferrochrome silicon the remaining 7 parts of high carbon chrome iron metal from the beneficiating step were to be added, there would be an exothermic mixture capable of producing 77 parts of ferrochrome analyzing 61.7 per cent chromium and 0.49 per cent carbon.

In reacting any of the described mixtures of oxidized and siliconized metal, a chrome-iron metal is formed in minute droplets which readily diffuse into a steel bath.

In the accompanying drawings, I have shown for purposes of illustration only, and not for purposes of limitation, flow sheets illustrating several of the possible chromium recovery processes which may be carried out in employing the principles of the invention. The flow sheets illustrate complete chromium recovery processes, commencing with the treatment of chromite ore initially and indicating the production ultimately of desirable chromium-bearing metal products.

Alternative methods of producing high-carbon ferrochromium are illustrated. Fig. 1 illustrates a process in which high-carbon ferrochromium is produced by direct reduction of the iron and chromium of chromite ore. Fig. 2 illustrates a process in which iron is selectively reduced from chromite ore with the production of a high-iron, low-chromium metal product and a beneficiated ore product, and the residual iron and chromium of the beneficiated ore product are reduced with carbon to produce high-carbon ferrochromium. In the process illustrated in Fig. 1, ferrochrome silicon is produced by smelting a portion of the high-carbon ferrochromium with carbon and silica, while in the process illustrated in Fig. 2, ferrochrome silicon is produced by smelting the high-iron, low-chromium metal product with carbon and silica. In dotted lines, I have suggested modified procedures which may employ oxidizing materials such as chromate, chlorate and nitrate compounds and alloying elements such as nickel, vanadium and molybdenum.

What I claim is:

1. A material made from chromite ore comprising oxidized ferrochromium substantially free of carbon in finely divided admixture with low carbon ferrochrome-silicon of a silicon content sufficient to reduce the metal oxides of said oxidized ferrochromium.
2. A silico-thermic material comprising in finely divided admixture oxidized ferrochromium substantially free of carbon, low carbon ferrochrome-silicon metal containing silicon in amount sufficient to reduce said oxidized ferrochromium to metal and lime in amount required to form a

basic silicate with the silica formed in said reduction.

3. A synthetic material composed of lime, ferric oxide, chromic oxide and chromium trioxide finely divided and in intimate admixture with ferrochrome silicon, said mixture being capable of undergoing internal reactions converting itself to chromium-iron metal and lime silicate slag.

4. A manufactured material useful in production of nickel-chromium-iron alloys by exothermic action which comprises a mixture of (1) a product in solid finely divided form mainly composed of oxides of iron and chromium in chemical combination with lime and formed by roasting carbon-bearing ferrochromium in the presence of lime to oxidize the metals and carbon of the ferrochromium and (2) solid finely divided nickel-ferrochrome silicon in quantity to reduce iron and chromium oxides contained in the roasted ferrochromium with formation of a lime-silicate slag.

5. A material manufactured from low grade chromite ore and comprising oxidized ferrochromium containing lime in chemical combination with chromic oxide and chromium trioxide in finely divided admixture with low carbon ferrochrome silicon of a chromium-iron ratio less than 1 and a silicon content about 40 per cent or less.

6. The method of producing a material suitable for use in the manufacture of alloys containing chromium and iron which comprises grinding a mixture of ferrochrome silicon and a product containing oxidized chromium formed by subjecting a carbon-bearing alloy containing iron and chromium to an oxidizing treatment, thereby to effect intimate mixing of finely divided particles of the ferrochrome silicon and finely divided particles of the product containing oxidized chromium.

7. A product suitable for use in the production of alloys containing chromium and iron comprising an intimate mixture of finely divided ferrochrome silicon and a product containing oxidized chromium formed by subjecting a carbon-bearing alloy containing iron and chromium to an oxidizing treatment, said intimate mixture being a product formed by grinding together the ferrochrome silicon and the product containing oxidized chromium.

8. The method of producing a reaction mixture suitable for use in the production of chromium alloys which comprises oxidizing carbon-bearing ferrochromium and forming an oxidized product low in carbon and containing iron and chromium in oxidized forms, and mixing the oxidized product in the solid state with solid, finely divided ferrochrome silicon.

9. The method of producing a reaction mixture suitable for use in the production of chromium alloys which comprises oxidizing carbon-bearing ferrochromium in a solid, finely divided condition and forming an oxidized product low in carbon and containing iron and chromium in oxidized forms, and mixing the oxidized product with solid, finely divided ferrochrome silicon.

10. The method of producing a reaction mixture suitable for use in the production of chromium alloys which comprises oxidizing carbon-bearing ferrochromium in a solid, finely divided condition and forming an oxidized product low in carbon and containing ferric oxide and chromic oxide, and forming a mixture containing (1) the ferric oxide and chromic oxide of the oxidized product, (2) solid, finely divided ferrochrome silicon and (3) oxidizing material capable of de-

veloping by reaction with silicon a temperature higher than those resulting from reaction of ferric oxide and chromic oxide with silicon.

11. The method of producing a reaction mixture suitable for use in the production of chromium alloys which comprises oxidizing carbon-bearing ferrochromium in a solid, finely divided condition and in the presence of lime and forming an oxidized product low in carbon and containing calcium oxide in chemical combination with chromium oxide, and mixing the oxidized product with solid, finely divided ferrochrome silicon.

12. The method of producing a reaction mixture suitable for use in the production of chromium alloys which comprises oxidizing carbon-bearing ferrochromium in a solid, finely divided condition and forming an oxidized product low in carbon and containing oxidized chromium a substantial amount of which is in the form of chromium trioxide, and mixing the oxidized product with solid, finely divided ferrochrome silicon.

13. The method of producing a reaction mixture suitable for use in the production of chromium alloys which comprises oxidizing carbon-bearing ferrochromium in a solid, finely divided condition and in the presence of lime and forming an oxidized product low in carbon and containing calcium oxide in chemical combination with oxidized chromium a substantial amount of which is in the form of chromium trioxide, and mixing the oxidized product with solid, finely divided ferrochrome silicon.

14. A reaction mixture suitable for use in the production of chromium alloys which comprises (1) oxidized ferrochromium in solid, finely divided condition produced by oxidizing carbon-bearing ferrochromium and forming a product low in carbon and containing iron and chromium in oxidized forms and (2) solid ferrochrome silicon.

15. A reaction mixture suitable for use in the production of chromium alloys which comprises (1) oxidized ferrochromium in solid, finely divided condition produced by oxidizing carbon-bearing ferrochromium in solid, finely divided condition and forming a product low in carbon and containing iron and chromium in oxidized forms and (2) solid ferrochrome silicon.

16. A reaction mixture suitable for use in the production of chromium alloys which comprises (1) oxidized ferrochromium in solid, finely divided condition produced by oxidizing carbon-bearing ferrochromium in solid, finely divided condition and forming a product low in carbon and containing ferric oxide and chromic oxide, (2) solid, finely divided ferrochrome silicon and (3) oxidizing material capable of developing by reaction with silicon a temperature higher than those resulting from reaction of ferric oxide and chromic oxide with silicon.

17. A reaction mixture suitable for use in the production of chromium alloys which comprises (1) oxidized ferrochromium in solid, finely divided form produced by oxidizing carbon-bearing ferrochromium in solid, finely divided condition and in the presence of lime and forming a product low in carbon and containing calcium oxide in chemical combination with chromium oxide and (2) solid, finely divided ferrochrome silicon.

18. A reaction mixture suitable for use in the production of chromium alloys which comprises (1) oxidized ferrochromium in solid, finely divided form produced by oxidizing carbon-bearing ferrochromium and forming a product low in carbon and containing iron oxide, chromic oxide

and a substantial amount of chromium trioxide and (2) solid, finely divided ferrochrome silicon.

19. A reaction mixture suitable for use in the production of chromium alloys which comprises (1) oxidized ferrochromium in solid, finely divided form produced by oxidizing carbon-bearing ferrochromium in solid, finely divided condition and in the presence of lime and forming a product low in carbon and containing calcium oxide in chemical combination with chromium oxide in which a substantial amount of the chromium is present in the form of chromium trioxide and (2) solid ferrochrome silicon.

20. A reaction mixture suitable for use in the production of metallic chromium by exothermic reaction, which comprises calcium chromite and calcium chromate intimately mixed with solid, finely divided ferrochrome silicon.

21. A reaction mixture suitable for use in the production of metallic chromium by exothermic reaction, which comprises calcium chromite, calcium chromate and sodium chromate intimately mixed with solid, finely divided ferrochrome silicon.

22. A reaction mixture suitable for use in the production of metallic chromium by exothermic reaction, which comprises calcium chromite and calcium chromate intimately mixed with a finely divided, solid ferrochrome silicon, the amount of chromium present in the mixture in the form of chromate being not substantially greater than the amount of chromium present in the mixture in the form of chromite.

23. A reaction mixture suitable for use in the production of metallic chromium by exothermic reaction, which comprises calcium chromite, calcium chromate and sodium chromate intimately mixed with a finely divided, solid ferrochrome silicon, the amount of chromium present in the mixture in the form of chromate being not substantially greater than the amount of chromium present in the mixture in the form of chromite.

24. A reaction mixture suitable for use in the production of a metallic chromium-bearing product by exothermic reaction which consists essentially of calcium oxide, ferric oxide, sodium oxide, chromic oxide and chromium trioxide intimately mixed with ferrochrome silicon, the amount of chromium present in the mixture in the form of chromium trioxide being not substantially greater than the amount of chromium present in the mixture in the form of chromic oxide.

25. A reaction mixture suitable for use in the production of metallic chromium by exothermic reaction, which comprises calcium chromite and calcium chromate intimately mixed with finely divided ferrochrome silicon, the amount of chromium present in the mixture in the form of chromate being not substantially greater than the amount of chromium present in the mixture in the form of chromite and the silicon and the oxygen available for reaction with the silicon being present in such amount and proportion that the mixture is capable upon ignition of converting itself by exothermic reaction into molten chromium-bearing metal and molten calcium silicate slag.

26. A reaction mixture suitable for use in the production of metallic chromium by exothermic reaction, which comprises calcium chromite, calcium chromate and sodium chromate intimately mixed with finely divided ferrochrome silicon, the amount of chromium present in the mixture in the form of chromate being not substantially greater than the amount of chromium present in

- the mixture in the form of chromite and the silicon and the oxygen available for reaction with the silicon being present in such amount and proportion that the mixture is capable upon ignition of converting itself by exothermic reaction into molten chromium-bearing metal and molten calcium silicate slag.
27. The method of producing a metallic alloy containing iron and chromium which comprises igniting a reaction mixture comprising (1) a product in the solid state produced by oxidizing carbon-bearing ferrochromium and forming an oxidized product low in carbon and containing iron and chromium in oxidized forms and (2) solid ferrochrome silicon.
28. The method of producing a metallic alloy containing iron and chromium which comprises igniting in contact with molten metal a reaction mixture comprising (1) a product in the solid state produced by oxidizing carbon-bearing ferrochromium and forming an oxidized product low in carbon and containing iron and chromium in oxidized forms and (2) solid ferrochrome silicon.
29. A method of producing a reaction mixture suitable for use in the production of chromium alloys which comprises reducing chromite ore with carbon to produce high-carbon ferrochromium, oxidizing the ferrochromium in solid, finely divided condition and forming an oxidized product low in carbon and containing iron and chromium in oxidized forms, smelting high-carbon ferrochromium with carbon in the presence of silica to produce low-carbon ferrochrome silicon, and mixing the oxidized product and the ferrochrome silicon in finely divided forms.
30. A method of producing a reaction mixture suitable for use in the production of chromium alloys which comprises reducing chromite ore with carbon to produce high-carbon ferrochromium, oxidizing a portion of the ferrochromium in solid, finely divided condition and forming an oxidized product low in carbon and containing iron and chromium in oxidized forms, smelting another portion of the ferrochromium with carbon in the presence of silica to produce low-carbon ferrochrome silicon, and mixing the oxidized product and the ferrochrome silicon in finely divided forms.
31. A method of producing a reaction mixture suitable for use in the production of chromium alloys which comprises smelting ferrous chromite ore in the presence of lime and a limited amount of carbon to selectively reduce iron and produce (1) a metal product high in iron and low in chromium and (2) a beneficiated ore product low in iron and high in chromium, smelting the beneficiated ore product with carbon to produce high-carbon ferrochromium, smelting the high-iron low-chromium product with carbon in the presence of silica to produce low-chromium low-carbon ferrochrome silicon, oxidizing the high-carbon ferrochromium in solid, finely divided condition and forming an oxidized product low in carbon and containing iron and chromium in oxidized forms, and mixing the ferrochrome silicon and the oxidized product in finely divided forms.

MARVIN J. UDY. 25